

# UNITED STATES PATENT OFFICE.

THOMAS JOHN IRELAND CRAIG, OF MANCHESTER, ENGLAND, ASSIGNOR OF ONE-HALF TO WHIPP BROS. & TOD, LIMITED, OF MANCHESTER, ENGLAND.

## FIREPROOFING OF TEXTILE FABRICS AND OTHER POROUS ARTICLES.

1,397,858.

Specification of Letters Patent.

Patented Nov. 22, 1921.

No Drawing.

Application filed October 30, 1917. Serial No. 199,260.

To all whom it may concern:

Be it known that I, THOMAS JOHN IRELAND CRAIG, a subject of the King of Great Britain and Ireland, and a resident of West Didsbury, Manchester, in the county of Lancaster, England, have invented certain new and useful Improvements in the Fireproofing of Textile Fabrics and other Porous Articles, of which the following is a specification.

10 This invention relates to the fireproofing of textile fibers and fabrics and other porous or absorbent substances or articles, and is an improvement in or modification of the invention described in the specification of 15 Patent No. 1,225,414.

In the specification of the said patent, there is described, *inter alia*, a treatment with acid alkali carbonate liquor of textile fibers and fabrics and other porous or absorbent substances or articles (hereinafter in this description and the appended claims for convenience referred to as fabric) which have been previously impregnated with suitable alkaline aluminates. The said treatment consists in immersing the aluminated fabric in acid alkali carbonate for a suitable time.

I have now found that I am able to obtain the desired effect of fixing the fireproofing body in the fabric by simply wetting the aluminated and preferably dried fabric with acid alkali metal carbonate solution and then subjecting it to a treatment at about 100° C. for a suitable time with steam or 30 with steam and carbon dioxide gas. When 35 treating the aluminated and dried fabric with acid alkali metal carbonate solution, I take care to maintain the latter in an acid condition by the addition of further acid 40 alkali metal carbonate, or by passing into it carbon dioxide gas either in the wetting out machine or in a subsidiary vessel; a circulation of liquor being suitably kept up between the wetting out machine and the 45 subsidiary vessel in the latter case. Before wetting the aluminated fabric with acid alkali metal carbonate solution, I may subject it to intermediate treatment, as described in the specification of Patent No. 1,225,414.

50 The following is an example of the manner in which I may carry out this alternative process forming the present invention:

Flannelette is impregnated with sodium aluminate, as described in the specification 55 of the aforesaid patent, and dried. The

dried aluminated fabric is then wetted out by suitable known means with hot concentrated acid sodium carbonate solution and squeezed to remove excess of liquor. The fabric is then subjected by known means 60 to a treatment with steam at about 100° C. for a suitable time, after which it may be washed and suitably dealt with in any desired manner.

According to a modification, the aluminated fabric, after being wetted out with the acid sodium carbonate solution and squeezed to remove the excess of liquor, is subjected to a treatment with steam and carbon dioxide gas at about 100° C. for a 70 suitable time.

I may carry out the herein described operation in or by any convenient means and in any convenient manner, and I do not confine myself to the precise details of the 75 operations hereinbefore mentioned, which are given merely by way of example.

What I claim as my invention and desire to secure by Letters Patent is:—

1. The process of rendering fibrous or absorbent materials and the like less inflammable, which consists in first treating said materials with an aluminate of an alkali metal, then subsequently treating said materials with a solution containing sodium bicarbonate, and finally subjecting said materials to heat.

2. The process of rendering fibrous or absorbent materials and the like less inflammable, which consists in first treating said materials with an aluminate of an alkali metal, then subsequently treating said materials with a solution containing sodium bicarbonate, and finally subjecting said materials to steam.

3. The process of rendering fibrous or absorbent materials and the like less inflammable, which consists in first treating said materials with an aluminate of an alkali metal, then subsequently treating said materials with a solution containing sodium bicarbonate, and finally subjecting said materials to steam at about 100° C.

4. The process of rendering fabrics and the like less inflammable, which consists in treating the fabric with an aluminate of an alkali metal, drying the same, treating the dried fabric with an acid alkali metal carbonate solution, and then subjecting the fabric to 105 the action of steam.

5. The process of rendering fibrous or absorbent materials and the like less inflammable, which consists in first treating said materials with an aluminate of an alkali metal, then subsequently treating said materials with a solution containing sodium bicarbonate, and finally subjecting the fabric to steam and carbon dioxide.
6. The process of rendering fibrous or absorbent materials and the like less inflammable, which consists in first treating said materials with an aluminate of an alkali metal, then subsequently treating said materials with a solution containing sodium bicarbonate, and finally subjecting the fabric to steam and carbon dioxide at substantially 100° C.
7. The process of rendering fabrics and the like less inflammable, which consists in treating the fabric with an aluminate of an alkali metal, drying the same, treating the dried fabric with an acid alkali metal carbonate solution, and then subjecting the fabric to the action of steam and carbon dioxide.
8. The process of rendering fabrics and the like less inflammable, which consists in first treating the fabric with a solution of sodium aluminate, then with a solution of sodium bicarbonate, and then subjecting the fabric to the action of steam.
9. The process of rendering fabrics and the like less inflammable, which consists in first treating the fabric with a solution of sodium aluminate, then with a solution of sodium bicarbonate, and then subjecting the fabric to the action of steam and carbon dioxide.
10. The process of rendering fabrics and the like less inflammable, which consists in first treating the fabric with a solution of sodium aluminate, then with a solution of sodium bicarbonate, and then subjecting the fabric to the action of steam at substantially 100° C.
11. The process of rendering fibrous or absorbent materials, and the like less inflammable, which consists in first impregnating said materials with an alkali aluminate, then treating said materials with an acid alkali metal carbonate, and then subjecting the same to the action of steam.
12. The process of rendering fibrous or absorbent materials, and the like less inflammable, which consists in first impregnating said materials with an alkali aluminate, then
- treating said materials with an acid alkali metal carbonate, and then subjecting the same to the action of steam and carbon dioxide.
13. The process of rendering fibrous or absorbent materials, and the like less inflammable, which consists in first impregnating said materials with an alkali aluminate, then treating said materials with an acid alkali metal carbonate, and then subjecting the same to the action of steam at substantially 100° C.
14. The process of rendering fibrous or absorbent materials, and the like less inflammable, which consists in first impregnating said materials with an alkali aluminate, then treating said materials with an acid alkali metal carbonate, and then subjecting the same to the action of steam and carbon dioxide at substantially 100° C.
15. The process of rendering substances less inflammable which consists in first treating the substances with an alkali aluminate, then wetting out the same with an acid alkali metal carbonate solution, removing the excess wetting liquid, and finally subjecting the substances to the action of steam.
16. The process of rendering substances less inflammable which consists in first treating the substances with an alkali aluminate, then wetting out the same with an acid alkali metal carbonate solution, removing the excess wetting liquid, and finally subjecting the substances to the action of steam at substantially 100° C.
17. The process of rendering substances less inflammable which consists in first treating the substances with an alkali aluminate, then wetting out the same with an acid alkali metal carbonate solution, removing the excess wetting liquid, and finally subjecting the substances to the action of steam and carbon dioxide gas.
18. The process of rendering substances less inflammable which consists in first treating the substances with an alkali aluminate, then wetting out the same with an acid alkali metal carbonate solution, removing the excess wetting liquid, and finally subjecting the substances to the action of steam and carbon dioxide gas with the temperature at substantially 100° C.

In witness whereof I have hereunto set my hand.

THOMAS JOHN IRELAND CRAIG.